

Sept. 16, 1969

M. WAYMAN ET AL

3,467,575

PROCESS OF BLEACHING PAPER WITH PERACETIC ACID

Filed Aug. 2, 1965

9 Sheets-Sheet 1



FIG. 1

MORRIS WAYMAN  
WILLIAM H. RAPSON  
INVENTORS

BY *Harold G. Fox*  
Attorney

Sept. 16, 1969

M. WAYMAN ET AL

3,467,575

PROCESS OF BLEACHING PAPER WITH PERACETIC ACID

Filed Aug. 2, 1965

9 Sheets-Sheet 2



FIG. 2

Morris Wayman  
William H. Rapson  
INVENTORS

BY *Harold G. Jor*  
Attorney

Sept. 16, 1969

M. WAYMAN ET AL

3,467,575

PROCESS OF BLEACHING PAPER WITH PERACETIC ACID

Filed Aug. 2, 1965

9 Sheets-Sheet 3



FIG. 3

MORRIS WAYMAN  
WILLIAM H. RAPSON  
INVENTORS

BY *Harold J. Fox*  
Attorney

Sept. 16, 1969

M. WAYMAN ET AL

3,467,575

PROCESS OF BLEACHING PAPER WITH PERACETIC ACID

Filed Aug. 2, 1965

9 Sheets-Sheet 4



FIG. 4

MORRIS WAYMAN  
WILLIAM H. RAPSON  
INVENTORS

BY *Darold J. Sox*  
Attorney

Sept. 16, 1969

M. WAYMAN ET AL

3,467,575

PROCESS OF BLEACHING PAPER WITH PERACETIC ACID

Filed Aug. 2, 1965

9 Sheets-Sheet 5



FIG. 5

MORRIS WAYMAN  
WILLIAM H. RAPPON  
INVENTORS

BY *Daniel J. Fox*  
Attorney

Sept. 16, 1969

M. WAYMAN ET AL

3,467,575

PROCESS OF BLEACHING PAPER WITH PERACETIC ACID

Filed Aug. 2, 1965

9 Sheets-Sheet 6



FIG. 6

Morris Wayman  
William H. Raason  
INVENTORS

BY *David G. Orr*  
Attorney

Sept. 16, 1969

M. WAYMAN ET AL

3,467,575

PROCESS OF BLEACHING PAPER WITH PERACETIC ACID

Filed Aug. 2, 1965

9 Sheets-Sheet 7



FIG. 7

Morris Wayman  
William H. Papson  
INVENTORS

BY *Barold G. Fox*  
Attorney

Sept. 16, 1969

M. WAYMAN ET AL

3,467,575

PROCESS OF BLEACHING PAPER WITH PERACETIC ACID

Filed Aug. 2, 1965

9 Sheets-Sheet 8



FIG. 8

Morris Wayman  
William H. Rapson  
INVENTORS

BY *Harold G. Ede*  
Attorney

Sept. 16, 1969

M. WAYMAN ET AL

3,467,575

PROCESS OF BLEACHING PAPER WITH PERACETIC ACID

Filed Aug. 2, 1965

9 Sheets-Sheet 9



FIG. 9

MORRIS WAYMAN  
WILLIAM H. RAPSON  
INVENTORS

BY *Harold E. Jr.*  
Attorney

1

3,467,575

**PROCESS OF BLEACHING PAPER WITH PERACETIC ACID**

Morris Wayman and William H. Rapson, Toronto, Ontario, Canada, assignors, by mesne assignments, to Hooker Chemical Corporation, Niagara Falls, N.Y., a corporation of New York

Filed Aug. 2, 1965, Ser. No. 476,452

The portion of the term of the patent subsequent to Oct. 1, 1985, has been disclaimed

Claims priority, application Great Britain, Aug. 13, 1964, 33,090/64

Int. Cl. D21h 3/80; D06l 3/00; D21c 9/16

U.S. Cl. 162—78

4 Claims

**ABSTRACT OF THE DISCLOSURE**

There are provided novel, economical processes for the bleaching of paper wherein bleached papers with excellent brightness and color reversion properties are obtained. In one of these processes, the paper is treated with up to about 2 percent of hydrosulphite (by weight) and then it is heated. In another of these processes, the paper is treated with from about 0.1 to about 2.6 percent of peracetic acid (by weight), heated to accelerate the bleaching reaction, and treated to neutralize the peracetic acid on the paper. In yet another of these processes the paper is treated with from about 0.1 to about 2.6 percent of peracetic acid, heated, treated with up to about 2 percent of hydrosulphite, and heated again.

This invention relates to the bleaching of paper.

In the manufacture of paper an important step is the bleaching of the fibres which will constitute the finished product. As far as we are aware, this operation is always carried out on the wood pulp. It requires mixing a pulp of high consistency with several liquids in succession, and holding the mixture of pulp and liquid in each case for several hours. A very large plant is required for these operations.

It is common practice in the manufacture of textiles to bleach the fabric rather than the unwoven fibres. The physical properties of the fabric are such that it will withstand the handling involved in impregnating and agitating it with successive bleaching and washing media. Such treatment would be impossible with paper, and no commercial process for bleaching paper has come into use in spite of the fact that a process for bleaching paper is described in Canadian Patent No. 461,242 to R. L. McEwan and F. R. Sheldon issued Nov. 22, 1949.

The bleaching of papermaking fibres as pulp is a well developed art which began when the use of rags in papermaking became widespread and which continued when the fibre base of paper changed to wood pulp.

For the bleaching of wood pulp for conversion into paper a very large plant is required, as mentioned hereinbefore. A typical modern pulp mill bleachery occupies 1,000,000 cubic feet of building space, and, with its contained equipment, may cost in the order of \$6,000,000.00. Several operations are required during each shift, and the time and attention of foremen, supervisors, chemists, quality control testers, engineers, maintenance men, research scientists, etc., are required to bleach wood pulp in a modern mill. The typical cost of bleaching chemicals is \$12.00 to \$16.00 per ton of pulp, and the total cost of bleaching pulp including capital expenditure, labour, power and supplies may amount to more than twenty percent of the selling price of the product.

It is evident that a process for bleaching paper which would avoid the necessity of a large bleachery and the

2

forementioned costs would represent an important advance in the industry.

In accordance with this invention, we have discovered certain processes, which are set out in detail hereinafter, by the practice of which paper can be bleached, thus eliminating the need for a bleachery for bleaching wood pulp fibres prior to their formation into paper.

Pulp sheets intended for later conversion into paper regularly are bleached by spraying with peroxide, and paper is regularly whitened by adding fillers of high brightness, or white or fluorescent dyes, or by applying coatings of higher brightness than the base stock.

It should be noted that our invention does not rely on the use of fillers, dyes or coatings to increase the brightness of paper. On the contrary, our processes involve the bleaching of paper, and by the term "bleaching" we mean a step which effects a chemical and physical change in paper affecting the fibres making up the paper and resulting in higher brightness. The term "brightness" as used herein refers to the reflectivity of paper measured with a "Zeiss," "Elrepho" (trademarks) brightness meter using a 457 millimicron filter and standardized against magnesium oxide. This measurement is the standard adopted by the Scandinavian Paper Engineers Association, and it is used in many pulp and paper mills and laboratories in North America, on the European Continent and elsewhere throughout the world, and corresponds to the TAPPI standard G.E. brightness.

As aforementioned, Canadian Patent No. 461,242 discloses a method of bleaching paper with peracetic acid. In this patent there is described a bleaching procedure in which an aqueous solution containing peracetic acid is applied to a web or sheet, and it is indicated that a brightness increment of 7.0 units is obtained, even though less than 1 percent of peracetic acid is used. This represents a significant and economical improvement. To the best of our knowledge, however, this process was never adopted in any commercial installation, and therefore has fallen short of achieving the highly desirable object of a commercial process for bleaching paper.

We have found that when paper is bleached in accordance with the process disclosed in this patent, the brightness increment claimed is obtained, but the colour of the bleached paper is not stable. Upon subjection of the treated paper to the standard heat-aging, brightness stability test, consisting of heating the paper in a circulated air oven at 105° C. for 18 hours, the brightness deteriorated, and, indeed, the bleached paper was found to have a poorer brightness than the unbleached paper after both had been aged.

In accordance with our invention, we have discovered processes for bleaching paper by virtue of which bleached papers of good brightness stability may be obtained.

It is a well-known fact that the "two-sidedness" of paper, meaning the difference in brightness between the felt side and the wire side of paper, particularly newsprint, has been a serious problem in the industry.

In accordance with this invention, we have discovered a process which not only offers the foregoing advantages, but also by the practice of which the problem of "two-sidedness" can be very materially reduced.

The processes which we have discovered for bleaching paper can be regarded in three groups: the first group involving the use of peracetic acid, the second group involving the use of hydrosulphites, and the third group involving the use of both peracetic acid and hydrosulphites. These processes will be described hereinafter with reference to the appended drawings in which:

FIGURE 1 is a graph depicting the effect on brightness, before and after aging, of neutralising the bleaching agent with various neutralising agents after the peracetic acid bleaching of newsprint and after heating of the

bleached newsprint, and the effect of varying amounts of peracetic acid picked up by the paper,

FIGURE 2 is a graph showing the effect of pH on the brightness of newsprint bleached with peracetic acid before and after aging and with and without after treatments,

FIGURE 3 is a graph illustrating the effect on brightness of the duration of the heating period when different papers bleached with peracetic acid were heated after bleaching and were subsequently neutralised with an  $\text{SO}_2$  solution,

FIGURE 4 is a graph indicating the effect on "twosidedness" of the duration of the heating period when different papers bleached with peracetic acid were heated after bleaching and were subsequently neutralised with an  $\text{SO}_2$  solution,

FIGURE 5 is a graph showing the effect on brightness of metabisulphite concentration in a solution used to neutralise the bleach in newsprint bleached with peracetic acid,

FIGURE 6 is a graph illustrating the effect on brightness, before and after aging, of varying amounts of different hydrosulphites picked up by newsprint in processes involving the bleaching of newsprint by hydrosulphites,

FIGURE 7 is a graph showing the effect on brightness, before and after aging, of pH and buffer concentration in processes involving the bleaching of newsprint by zinc hydrosulphite,

FIGURE 8 is a graph indicating the effect on brightness, before and after aging, of the duration of a heating period which follows the zinc hydrosulphite bleaching of newsprint, and

FIGURE 9 is a graph indicating the effect on brightness, before and after aging, of a number of different conditions in the bleaching of newsprint with peracetic acid followed by zinc hydrosulphite.

#### General

Each of the processes to be described in detail hereinafter involves the application of a bleaching agent to paper. The bleaching agent is applied from an aqueous solution of the bleaching agent, buffered if necessary. The bleaching solution may be applied in any number of ways, e.g., by dipping the paper in the bleaching solution, by running the paper continuously through the bleaching solution, by padding with applicator rolls, by spraying, etc.

Most of the processes to be described in detail herein-after involve the application of heat to the bleached paper. The purpose of the heating step is to accelerate the bleaching reaction. The degree of acceleration of the bleaching reaction is dependent on both time and temperature. It may be desirable to employ temperatures which permit the heating period to be as short as possible, but in all cases care must be taken to ensure that the times and temperatures which are selected will not result in discolouring of the paper, this being within the province of those skilled in the art.

The heat may be applied in a number of ways, as, for example, by clamping the paper between heated plates. For continuous operation it is contemplated that dielectric heating may be employed. Generally speaking it would be undesirable to heat the bleached paper above the steam point, i.e. 100° C. at normal pressures.

An important feature of a number of the processes set out hereinafter is the neutralising of the bleaching agent on the paper. Many types of neutralising agents may be employed. Generally the neutralising agents will be applied from aqueous solutions thereof, and the mode of application may be the same as for the solutions of bleaching agents.

Where herein we refer to percentages of bleaching agent on paper or being picked up by paper, e.g., 1% peracetic acid on paper, this is a weight percentage based on the weight of the dry paper.

It should be noted that pH values given in the following examples are measured in the solution before application to the paper.

Where reference is made herein to the unqualified term "newsprint," this refers to commercial newsprint obtained from a source in Eastern Canada and made of sulphite and groundwood in conventional proportions, primarily of spruce-balsam.

In the following examples sheets of paper were cut to 10 cm. x 20 cm., and 10 cm. of each sheet was dipped in distilled water in a shallow tray. The paper was then passed upwards between a pair of rubber rollers under pressure to wring out the water from the wet half of the paper. The wet half of the paper then contained about 67 percent moisture, 33 percent fibre. The dry half of the paper acted as control.

A series of shallow plastic photographic trays was used for applying bleach. Bleach solutions were made up in the trays. Insofar as possible, buffers or other chemicals were added to the water in the trays and the pH adjusted, based on experience, before the bleaching agent itself was added. The purpose of this sequence was to minimize the time between preparation and use of bleach solutions. Before use, the bleach was analysed. Most experiments were carried out at the room temperature. To apply the bleach, the sheet was weighed, the wet half of the sheet was held immersed in the bleach solution, usually for 30 seconds, then passed through the wringer to remove excess bleach. The pH and residual bleach in the solution then were increased. A thin strip of paper was cut off and coiled in a beaker of distilled water for pH measurement.

In most experiments the paper, wet with bleach, was put between the two 10 cm. x 10 cm. heated plates of a Carver press, the plates being at a controlled temperature of 100° C.

In many of the experiments involving bleaching, the sheets, after removal from the heated press, were dipped into a second bath for an after treatment, usually with  $\text{SO}_2$  solution or sodium metabisulphite, but occasionally with water or with other chemicals. They were again passed through the wringer, air dried in the constant temperature-constant humidity room, and tested by standard procedures.

#### Peracetic acid bleaching of newsprint

It has been discovered that paper may be bleached quite successfully by a process which involves the steps of applying peracetic acid to the paper, thereafter heating the bleached paper to accelerate the bleaching reaction, and subsequently neutralising the residual bleaching agent on the paper. This process is described in the following examples.

#### Example I

Peracetic acid solutions containing 0-20 grams/liter (in this procedure 7.5 g.p.l. solution is equivalent to 1% bleach on paper) together with a mixed silicate-phosphate buffer containing 7.5 g.p.l. of sodium tetracyanophosphate and 4.0 g.p.l. of sodium silicate were applied to newsprint with the pH adjusted to 8.0 in the case of the metabisulphite series and 9.0 for the  $\text{SO}_2$  and water series. The treated paper was heated in a press at 100° C. for 20 seconds, this step being followed by an after treatment by virtue of which either water, an  $\text{SO}_2$  solution of pH 3, or a 7.5 g.p.l. sodium metabisulphite solution at pH 4.3 was applied to the paper to neutralise the residual bleaching agent. The paper subsequently was aged in a circulated air oven at 105° C. for 18 hours.

The results obtained are shown in FIGURE 1. The brightness of the paper increased regularly with increasing ratios of peracetic acid, such that the newsprint originally at 57 brightness was raised to 64-65 brightness by 0.5% peracetic acid on paper, and to 67-69 brightness with 1% peracetic acid on paper. When  $\text{SO}_2$  or water was used as an after treatment, the brightness rose slowly as the peracetic acid solution was increased but did

not quite reach 70 even with 2.6% peracetic acid on the paper.

Best results were obtained by using sodium metabisulphite to ensure adequate reducing power to destroy residual bleach and to lower pH in a controlled fashion. The metabisulphite had some bleaching ability of its own, and it can be seen from FIGURE 1 that the control, shown at 0% peracetic acid, which had exactly the same treatment as all other papers, except that the buffer solution contained no peracetic acid, had a brightness of 59.8 after treatment, whereas the untreated paper had a brightness of 57.8, the 2 point increase being attributable to the sodium metabisulphite. When  $\text{SO}_2$  was used it contributed about 1 unit brightness increase to paper not treated with peracetic acid.

When sodium metabisulphite was used for the after treatment, the brightness of the paper continued to increase at higher levels of peracetic acid on the paper at a rate of about 3.5 units per 1% peracetic acid and 75 brightness was reached with 2.5% peracetic acid on the paper.

The brightness of the paper after aging was retained quite well with both water and  $\text{SO}_2$  after treatments up to about 1% peracetic acid on the paper, but fell off at higher ratios, whereas, when sodium metabisulphite was used as the after treatment, the aged brightness remained satisfactory at higher percentages of peracetic acid on the paper. The water treatment was less effective than  $\text{SO}_2$  treatment in controlling colour reversion on aging. The P.C. numbers are given in Table I where the P.C. 30 number is the post colour number.

$$= \frac{100(1-Ba)^2}{2Ba} - \frac{(1-B)^2}{2B}$$

In the above formula, B=brightness and Ba=brightness 35 after aging.

TABLE I

| Peracetic acid (percent on paper) | Brightness   |             |          |
|-----------------------------------|--------------|-------------|----------|
|                                   | Before aging | After aging | P.C. No. |
| 0 untreated.....                  | 57.8         | 54.3        | 3.82     |
| 0 control.....                    | 59.8         | 55.1        | 4.78     |
| Metabisulphite series:            |              |             |          |
| 0.1.....                          | 64.2         | 58.4        | 4.84     |
| 0.2.....                          | 65.5         | 59.7        | 4.51     |
| 0.4.....                          | 65.4         | 59.5        | 4.63     |
| 0.8.....                          | 68.2         | 62.0        | 4.24     |
| 1.1.....                          | 69.0         | 62.4        | 4.36     |
| 1.2.....                          | 71.6         | 63.2        | 5.09     |
| 1.8.....                          | 72.2         | 63.8        | 4.92     |
| 2.2.....                          | 72.7         | 64.1        | 4.92     |
| 2.5.....                          | 75.0         | 65.7        | 4.78     |
| $\text{SO}_2$ series:             |              |             |          |
| 0 control.....                    | 58.9         | 56.2        | 2.7      |
| 0.13.....                         | 60.2         | 56.8        | 3.3      |
| 0.20.....                         | 61.3         | 58.3        | 2.7      |
| 0.36.....                         | 62.9         | 58.9        | 3.4      |
| 0.39.....                         | 63.2         | 59.9        | 2.7      |
| 0.53.....                         | 64.2         | 59.9        | 3.4      |
| 0.70.....                         | 65.9         | 61.3        | 3.4      |
| 0.83.....                         | 66.4         | 61.6        | 3.5      |
| 1.12.....                         | 66.6         | 60.8        | 5.8      |
| 1.13.....                         | 68.2         | 63.4        | 3.2      |
| 1.36.....                         | 67.1         | 60.3        | 5.0      |
| 1.38.....                         | 68.4         | 61.6        | 4.7      |
| 1.59.....                         | 68.7         | 61.1        | 5.3      |
| 2.62.....                         | 69.4         | 59.2        | 7.3      |
| Water series:                     |              |             |          |
| 0 control.....                    | 57.8         | 54.5        | 3.6      |
| 0.13.....                         | 59.5         | 56.0        | 3.5      |
| 0.20.....                         | 60.8         | 57.5        | 3.1      |
| 0.36.....                         | 62.5         | 58.2        | 3.8      |
| 0.39.....                         | 62.6         | 58.3        | 3.7      |
| 0.53.....                         | 63.3         | 58.6        | 4.0      |
| 0.70.....                         | 65.1         | 59.9        | 4.1      |
| 0.83.....                         | 65.8         | 60.4        | 4.1      |
| 1.12.....                         | 66.7         | 60.3        | 4.8      |
| 1.13.....                         | 67.6         | 61.9        | 4.0      |
| 1.36.....                         | 67.5         | 60.9        | 4.7      |
| 1.38.....                         | 68.2         | 60.8        | 5.2      |
| 1.59.....                         | 68.6         | 61.2        | 5.1      |
| 2.62.....                         | 69.5         | 58.6        | 7.9      |

It can be seen from Table I that the brightness stability, as measured by the P.C. number, remains about the same as for untreated paper and is in a range which would be considered acceptable.

## Example II

In this example, which demonstrates the effect of the pH of the bleaching solution on brightness, newsprint was treated with an 8.5 g.p.l. peracetic acid solution (1.2% on the paper) at varying pH in a buffer containing 4.0 g.p.l. sodium silicate and 7.5 g.p.l. sodium tetrabyphosphate. In some cases the bleach was not neutralised after heating, whereas in other cases an after treatment using an  $\text{SO}_2$  solution of pH 3 was carried out. 10 The treated paper was heated for 20 seconds between plates at 100° C., and aging conditions were at 105° C. for 18 hours.

The results are shown in FIGURE 2. It can be seen from FIGURE 2 that there was no marked trend in the brightening effect attributable to pH, although a slight maximum occurs between pH's 8 and 9. However, as shown in FIGURE 2, brightness stability was sharply affected by the pH of the peracetic acid treatment. Best results were obtained with a pH of 8.

## Example III

In this example, which demonstrates the effect of the duration of the heating period, 1.2% peracetic acid on the paper was obtained from an aqueous peracetic acid solution containing a mixed buffer consisting of 7.5 g.p.l. of sodium tetrabyphosphate and 4.0 g.p.l. of sodium silicate, the pH of the solution being 9.0. The treated paper, newsprint, Rotonews and Directory, was heated for varying intervals between plates at 100° C. and an after treatment with  $\text{SO}_2$  solution at pH 3 was employed. The Rotonews contained 27% sulphite, while the Directory paper was 43% sulphite, the remainder in both cases being groundwood with a small percentage of filler.

The results are shown in FIGURE 3. Examination of FIGURE 3 reveals a slight maximum after 15 seconds' heating, with best results being obtained for heating period of 15-20 seconds between plates at 100° C. It should be noted that the brightness values indicated in FIGURE 3 are the average of the two sides of the paper sheet. Best results were obtained with Directory paper, Rotonews being second and newsprint third.

## Example IV

In this example, which demonstrates the effect of the process on the "two sidedness" of newsprint, the same bleached papers as used in Example 3 were employed.

It will be seen from FIGURE 4, where the results of this process are shown, that a sharp reduction in the "two sidedness" of the newsprint was obtained, best results occurring for papers heated between 10 and 30 seconds. The improvement in the newsprint was most marked. For untreated newsprint the difference in brightness of the two sides was about 2.4 units, and in the best case, this was reduced to 0.2 unit after about 10 seconds' heating.

## Example V

In this example, which demonstrates the effect of metabisulphite concentration on brightness, the conditions were as follows: 1.1% peracetic acid on newsprint obtained from an aqueous solution of peracetic acid containing 4 g.p.l. sodium silicate and 7.5 g.p.l. sodium tetrabyphosphate buffer at pH 8.0, heating for 20 seconds between plates at 100° C. followed by metabisulphite treatment at varying concentrations.

The results obtained are shown in FIGURE 5. It will be seen that the bleached newsprint brightness obtained increased with increasing concentration of sodium metabisulphite up to about 8 g.p.l. where brightness levelled off. In one case the paper was not treated with peracetic acid, and the lower curve in FIGURE 5 was obtained, which indicates that sodium metabisulphite has some bleaching action by itself. The increase in brightness in this case was about two units, the original brightness of 57.4 being raised to 59.9 by 8 g.p.l. sodium metabisulphite as the only treatment. In the case where peracetic

acid was employed, the increase in brightness was about 4 units.

#### SUMMARY

From the foregoing it can be seen that the best conditions for bleaching newsprint with peracetic acid were found in these experiments to be:

(a) Treatment of the moist paper with a peracetic acid solution buffered to pH 8 to 9, the buffer being made up of sodium silicate and sodium tetrapyrophosphate, followed by

(b) Heating in a press at 100° C. for 15 to 20 seconds, and then

(c) An after treatment with sodium metabisulphite solution.

Under these conditions, newsprint of 57 brightness was raised to 65 brightness with 0.25 percent peracetic acid on paper, 70 brightness with 1.2 percent peracetic acid on paper, and 75 brightness with 2.5 percent peracetic acid on paper. The bleached paper had an acceptable P.C. value under the severe aging conditions used in the test. Under the best conditions of bleaching, "two sidedness" was reduced and almost eliminated.

#### HYDROSULPHITE BLEACHING OF NEWSPRINT

It has been discovered that paper may be bleached quite successfully by a process which involves the application of aqueous hydrosulphite solutions to the paper. If desired, the treated paper may be heated to accelerate the bleaching reaction but, in contrast to peracetic acid bleaching, no neutralisation of the residual hydrosulphite bleach is required. Since heating is not necessary in this case, the paper may be air dried if desirable.

It is known to bleach pulp with hydrosulphite, sometimes in conjunction with a pretreatment with  $H_2O_2$  and  $SO_2$ , but, owing to the instability of the hydrosulphite, care always has been taken to keep it away from air. It is surprising that hydrosulphite will operate satisfactorily in a treatment of paper in which it is fully exposed to air, and that a treatment with this material alone is sufficient to produce good, comparatively stable brightness.

The following examples illustrate this process:

#### Example VI

Solutions of sodium or zinc hydrosulphite containing 0.1 M  $KH_2PO_4$  buffered at a pH of 6.0 were applied to newsprint with the amounts of hydrosulphite picked up by the paper being varied. The treated paper was heated between plates at 100° C. for 30 seconds. Aging was at 105° C. for 18 hours.

From the results shown in FIGURE 6, it can be seen that hydrosulphites are excellent bleaching agents for newsprint, brightness being raised from 57.7 to 65 by 0.4% of either sodium or zinc hydrosulphite on paper, with good brightness retention on aging. Higher ratios of zinc hydrosulphite resulted in higher brightness, 2.0 percent on paper resulting in 69 brightness. However, treated newsprint of brightness above 65 was not as stable to the aging test. Results with sodium hydrosulphite were somewhat erratic.

#### Example VII

In this example 10 g.p.l. zinc hydrosulphite solutions (equivalent to 1.4% hydrosulphite on paper) at variable pH's and containing 0.1 or 0.2 M.  $KH_2PO_4$  were applied to the newsprint. The treated papers were heated for 20 seconds between plates at 100° C. Aging conditions were as in Example 6.

The results are shown in FIGURE 7 which indicates that brightness was best at pH 4.0 to 5.0, that brightness stability was best at pH 5.0, and that buffer concentration has a significant effect on brightness, the more concentrated buffer resulting in 1.5 units higher brightness.

#### Example VIII

Example 7 was repeated using hydrosulphite solutions of pH 5.0 and containing 0.1 M  $KH_2PO_4$ . The treated

paper was heated for varying intervals between plates at 100° C.

The results obtained are shown in FIGURE 8. As may be seen by reference to this figure, best results were obtained with very short heating times of the order of 5 seconds. Heating for periods longer than 30 seconds resulted in losses in both brightness and brightness stability to aging.

The best conditions for bleaching newsprint with zinc hydrosulphite were found in these experiments to be:

(a) Treatment of the moist paper with zinc hydrosulphite solution buffered to pH 5.0, the buffer being 0.2 M  $KH_2PO_4$ , followed by

(b) Heating in a press at 100° C. for 5 to 30 seconds.

Newsprint of 57.5 brightness was raised to 65 brightness by bleaching with 0.4 percent zinc hydrosulphite on paper, and 69 brightness with 1.4 percent zinc hydrosulphite on paper. Sodium hydrosulphite was as effective as the zinc compound in raising the brightness of the newsprint to 65, but the results on addition of higher ratios of sodium hydrosulphite were erratic.

#### Multi stage bleaching of newsprint

It has been discovered that paper may be bleached quite successfully by a process which involves the steps of applying peracetic acid to the paper, heating the treated paper, followed by the application of a hydrosulphite, or by such a process where sodium metabisulphite is applied to the paper after treatment with peracetic acid and heating but before treatment with the hydrosulphite. Heating is not required after the hydrosulphite treatment and the paper may be air dried if desired. Heating of the paper after the hydrosulphite treatment is desirable, however, as is evidenced by FIGURE 8.

The preferred conditions for carrying out these multi-stage bleaching processes are as previously indicated in connection with the individual processes described in the previous examples.

It is known to bleach pulp using in sequence an alkali metal peroxygen compound, an acid sulphite or  $SO_2$  solution and a hydrosulphite, but the conditions of operation in the bleaching of pulp on the one hand and paper on the other are completely different, and for the aforementioned reasons, it would not have been expected that hydrosulphite could be used successfully for the latter.

The following example is illustrative of these multi-stage processes:

#### Example IX

Newsprint was treated with an aqueous solution of peracetic acid buffered with 4 g.p.l. sodium silicate and 7.5 g.p.l. sodium tetrapyrophosphate at pH 8.0. The pick up was 1% peracetic acid on to the weight of the paper. The treated paper was heated in a press at 100° C. for 20 seconds. In one case no after treatment was employed. In another case the paper was treated with a 7.5 g.p.l. sodium metabisulphite solution. In still another case the paper was treated with zinc hydrosulphite solutions buffered to pH 5.0 with 0.1 M  $KH_2PO_4$ . In still another case the paper was treated with both the sodium metabisulphite and zinc hydrosulphite solutions mentioned hereinbefore with the sodium metabisulphite treatment preceding the zinc hydrosulphite treatment. In the latter three cases the paper was heated in a press for 20 seconds at 100° C. In all cases aging was as in Example 8.

The results are shown in FIGURE 9.

It is evident from FIGURE 9 that the two stage bleach resulted in high brightness, the newsprint being raised from 57.6 to 75.3 by the use of 1.0 percent peracetic acid following by 1.2 percent zinc hydrosulphite on paper. The brightness stability to aging at 105° C. for 18 hours was satisfactory, P.C. numbers being in the range of 4.2 to 7.1.

At very low applications of zinc hydrosulphite, up to 0.2 percent on paper, the use of a sodium metabisulphite

intermediate stage was advantageous, and indeed the small amount of zinc hydrosulphite did not improve the brightness or brightness stability over the metabisulphite alone. This was in the brightness range up to 70, and this observation could be of some importance for newsprint bleaching. At high brightness levels, or high ratios of zinc hydrosulphite to paper, the sodium metabisulphite was not advantageous, and in fact resulted in somewhat lower brightness than the direct two stage peracetic acid-zinc hydrosulphite procedure.

Comparison with FIGURE 1 shows that 2.5 percent peracetic acid followed by 1.0 percent sodium metabisulphite was as effective as the best of these results in raising the brightness of the same newsprint, but at present the costs of chemicals are such that the two stage process with hydrosulphite would be advantageous. Hydrosulphite alone, as shown in FIGURE 6 did not achieve the same high level of brightness.

In addition to newsprint, thirteen other types of paper were bleached by the procedures discussed herein. The papers were mostly groundwood-containing papers, but unbleached kraft and high yield sulphite papers were included. Laboratory papers included newsprint made of groundwood and unbleached kraft pulp in place of the conventional semi-bleached kraft pulp. Four bleaching processes were used, peracetic acid, peroxide, zinc hydrosulphite and the two-stage peracetic acid-zinc hydrosulphite process. The results are shown in Table II.

bleached grade, the best brightness obtained being 36.2. However, the laboratory papers containing 20 percent unbleached kraft and 80 percent groundwood were raised to an acceptable newsprint brightness level by either peracetic acid or by zinc hydrosulphite when the groundwood was spruce, or by the two stage process when hemlock groundwood was used.

The refiner groundwood paper was brightened more by zinc hydrosulphite treatment than by peracetic acid treatment. The two stage process however, raised the brightness of this paper about 12 units.

The pine high yield sulphite paper was of very poor brightness (37.8) as received, and any of the processes improved it, but even the two stage process only raised the brightness to 51.7. The corresponding paper made of spruce began at 50.6 brightness and was raised by the two stage process to 61.3. Peracetic acid was considerably more effective than hydrosulphite in bleaching this paper. The spruce groundwood paper No. 12 responded well above average to all three processes, and was raised to 74.6 brightness from 61.5 by the two stage process. The laboratory paper, of which spruce groundwood formed 75 percent and high yield spruce sulphite the remainder, behaved as would have been expected, based on the behaviour of the two components, whereas the corresponding pine paper responded better than expected to all three processes, and particularly to the zinc hydrosulphite treatment and its brightness was raised by the two stage process from 53.4 to 70.1.

TABLE II.—PAPER BLEACHING

See legend following table for the meaning of the symbols.

(a) Paper Description.

No. Description  
 1—Newsprint, sulphite, groundwood  
 2—Rotonews A, sulphite, groundwood  
 3—Rotonews B, 27 percent sulphite, 73 percent groundwood  
 4—Directory, 44 percent sulphite, 56 percent groundwood  
 5—Kraft, West Coast coniferous.  
 6—Laboratory "news" 20 percent W.C. kraft, 80 percent hemlock g.w.  
 7—Laboratory "news" 20 percent W.C. kraft, 80 percent spruce g.w.  
 8—Refiner g.w. West Coast coniferous.

(b) Brightness after bleaching.

9—Laboratory "news" 10 percent W.C. kraft, 90 percent refiner g.w.  
 10—Sulphite, 68 percent yield, pine.  
 11—Laboratory paper, 25 percent pine H.Y. sulphite, 75 percent spruce g.w.  
 12—Spruce g.w.  
 13—Sulphite, 67 percent yield, spruce.  
 14—Laboratory paper, 25 percent spruce H.Y. sulphite, 75 percent spruce g.w.

| Paper No.    | Untreated |       |       | Peracetic acid |       |       | G     | Zinc Hydrosulfite |       |       | Two stage P.A.-Z.H. |       |       |       |       |
|--------------|-----------|-------|-------|----------------|-------|-------|-------|-------------------|-------|-------|---------------------|-------|-------|-------|-------|
|              | B         | Ba    | P C   | B              | Ba    | P C   |       | B                 | Ba    | P C   | G                   | B     | Ba    | P C   | G     |
| 1-----       | 57.6      | 54.7  | 3.15  | 69.0           | 63.1  | 3.83  | 11.4  | 67.5              | 60.7  | 4.90  | 9.9                 | 72.8  | 66.0  | 3.68  | 15.2  |
| 2-----       | 60.2      | 55.2  | 5.0   | 70.5           | 64.0  | 3.96  | 10.3  | 69.7              | 62.0  | 5.06  | 9.5                 | 72.9  | 66.8  | 3.3   | 12.7  |
| 3-----       | 61.8      | 59.1  | 2.4   | 73.0           | 67.2  | 3.02  | 11.2  | 72.5              | 65.3  | 4.00  | 10.7                | 75.8  | 69.1  | 3.0   | 14.0  |
| 4-----       | 65.0      | 60.9  | 3.2   | 74.8           | 69.1  | 2.66  | 9.8   | 73.6              | 66.9  | 3.45  | 8.6                 | 76.7  | 70.7  | 2.6   | 11.7  |
| 5-----       | 26.2      | 26.0  | ----- | 36.2           | 33.7  | ----- | 10.0  | 31.7              | 30.1  | ----- | 5.5                 | 35.3  | 33.3  | ----- | 9.1   |
| 6-----       | 46.4      | 43.9  | 4.89  | 56.9           | 52.2  | 5.57  | 10.5  | 53.3              | 49.4  | 5.45  | 6.9                 | 60.1  | 55.0  | 5.2   | 13.7  |
| 7-----       | 52.4      | 48.0  | 6.38  | 60.0           | 56.0  | 3.96  | 7.6   | 60.6              | 55.2  | 5.37  | 8.2                 | 63.6  | 57.8  | 5.0   | 11.2  |
| 8-----       | 56.3      | 51.6  | 5.74  | 63.7           | 55.9  | 7.06  | 7.4   | 66.0              | 55.7  | 8.86  | 9.7                 | 68.3  | 59.6  | 6.30  | 12.0  |
| 9-----       | 50.8      | 46.8  | 6.41  | 59.3           | 53.3  | 6.49  | 8.5   | 59.3              | 51.5  | 8.87  | 8.5                 | 62.5  | 56.2  | 5.82  | 11.7  |
| 10-----      | 37.8      | 35.2  | 8.47  | 48.1           | 44.9  | 5.81  | 10.3  | 49.5              | 42.5  | 13.14 | 11.7                | 51.7  | 45.0  | 11.05 | 13.9  |
| 11-----      | 53.4      | 50.8  | 3.50  | 64.5           | 59.9  | 3.65  | 11.1  | 66.0              | 59.3  | 5.21  | 12.6                | 70.1  | 62.9  | 4.50  | 16.7  |
| 12-----      | 61.5      | 59.0  | 2.20  | 71.9           | 66.1  | 3.20  | 10.4  | 72.2              | 65.2  | 3.94  | 10.7                | 74.6  | 68.6  | 2.77  | 13.1  |
| 13-----      | 50.6      | 48.0  | ----- | 58.1           | 54.3  | 4.12  | 7.5   | 56.1              | 49.5  | 8.58  | 5.5                 | 61.3  | 55.2  | 5.97  | 10.7  |
| 14-----      | 58.4      | 55.5  | 3.02  | 67.8           | 63.1  | 3.14  | 9.4   | 67.5              | 60.7  | 4.49  | 9.1                 | 70.9  | 65.5  | 3.12  | 12.5  |
| Average----- | -----     | ----- | ----- | -----          | ----- | 9.7   | ----- | -----             | ----- | ----- | 9.1                 | ----- | ----- | 12.7  | ----- |

B = Brightness; Ba = Brightness after aging at 105° C. for 18 hours; PC = P C number; G = Bleached brightness minus untreated Brightness ("Gain")  
 Peracetic Acid: 1.1 percent peracetic acid on paper, buffered to pH 8.0 with 4.0 g.p.l. sodium silicate and 7.5 g.p.l. sodium tetrapyrophosphate, heated between plates at 100° C. for 20 seconds, followed by 7.5 g.p.l. sodium metabisulphite.

Zinc Hydrosulfite: 1.2 percent zinc hydrosulfite on paper, buffered to pH 8.0 with 0.1 M KH<sub>2</sub>PO<sub>4</sub>, heated between plates at 100° C. for 20 seconds.

Two stage PA-ZH: 1.1 percent peracetic acid on paper, buffered to pH 8.0 with 4.0 g.p.l. sodium silicate and 7.5 g.p.l. sodium tetrapyrophosphate, heated between plates at 100° C. for 20 seconds, followed by 1.2 percent zinc hydrosulfite on paper, buffered to pH 5.0 with 0.1 M KH<sub>2</sub>PO<sub>4</sub>, heated between plates at 100° C. for 20 seconds.

The average brightness gain for this variety of papers bleached by these three processes are shown at the bottom of the G columns, the two stage peracetic acid-zinc hydrosulfite process resulting in an average brightness gain of 12.7 units, peracetic and metabisulphite 9.7 and zinc hydrosulfite 9.1. The process conditions were reasonably close to optimal for each process, as shown by the previous results for newsprint, but not necessarily optimal for each variety of paper.

The unbleached kraft paper, paper No. 5 was brightened most by peracetic acid, but was still below a semi-

65 Examination of the P.C. numbers shows that these processes did not, for the most part, adversely affect the brightness stability to aging of any of these papers, improving it in many cases.

70 Aside from brightness other properties of newsprint bleached by processes within the scope of this invention were examined. The following Table III indicated the results of colour tests made on newsprint bleached with 0.8 percent peracetic acid on paper (pH 9.0) followed by heating and an after treatment with an SO<sub>2</sub> solution at pH 3.

TABLE III.—OPTICAL PROPERTIES OF BLEACHED NEWSPRINT

|                                     | Untreated | Bleached |
|-------------------------------------|-----------|----------|
| Curve No.                           | 6725      | 6726     |
| Reflectance at 457 1/2 millimicrons | 0.556     | 0.663    |
| Reflectance at 570 millimicrons     | 0.678     | 0.819    |
| X                                   | 0.3328    | 0.3325   |
| Y                                   | 0.3410    | 0.3423   |
| Visual efficiency                   | 0.670     | 0.804    |
| Dominant wavelength                 | 576.4     | 575.6    |
| Percent saturation                  | 12.7      | 12.9     |
| Scattering coefficient (s)          | 0.093     | 0.096    |
| Absorption coefficient (k)          | 0.0074    | 0.0023   |
| Printing opacity (actual)           | 0.954     | 0.900    |
| Printing opacity (32 lb.)           | 0.949     | 0.889    |
| Basis wt.                           | 33.2      | 34.3     |

It will be seen that printing opacity has been somewhat reduced by the process, while the percent saturation is hardly changed, and while the dominant wavelength trends towards the blue, it does so to a less extent than normal than when pulps are bleached.

It is contemplated that the processes hereinbefore described may be carried out directly on a paper machine with the bleaching solution being applied at the wet end of the paper machine, the heat to accelerate the bleaching reaction being obtained in the dryer section and the neutralising solution, where required, being applied at some point between the beginning and end of the dryer section.

What we claim as our invention is:

1. A process for bleaching paper, which comprises:
  - applying to the paper from about 0.1 to about 2.6 percent of peracetic acid (by weight);
  - heating the treated paper at a temperature and for a time sufficient to accelerate the bleaching reaction between the peracetic acid and the paper, while being insufficient to discolor the paper; and
  - neutralizing the peracetic acid on the paper by application thereto of a compound selected from the

group consisting of sodium metabisulphite and sulfur dioxide.

2. The process of claim 1, wherein:

- the peracetic acid is in a buffered solution at a pH of from about 8 to about 9; and
- the treated paper is heated at a temperature of about 100° C. for from about 15 to about 20 seconds.

3. The process of claim 1, wherein the peracetic acid is in a buffered solution at a pH of about 8 to about 9, which buffered solution comprises sodium silicate and sodium tetrapyrophosphate.

4. The process of claim 2 wherein the buffered solution of peracetic acid comprises sodium silicate and sodium tetrapyrophosphate.

References Cited

UNITED STATES PATENTS

|           |         |                  |          |
|-----------|---------|------------------|----------|
| 3,085,039 | 4/1963  | Gartner          | 162—78   |
| 1,154,851 | 9/1915  | Foley            | 162—13   |
| 1,645,061 | 10/1927 | Kress            | 162—85   |
| 2,125,634 | 8/1938  | Heritage         | 162—13   |
| 2,150,926 | 3/1939  | Kauffmann et al. | 162—13   |
| 2,347,434 | 4/1944  | Reichert et al.  | 162—78 X |
| 2,492,047 | 12/1949 | Burg et al.      | 162—17   |
| 2,598,580 | 5/1952  | McEwen et al.    | 162—13   |
| 2,862,784 | 12/1958 | Kise et al.      | 162—78   |
| 2,963,395 | 12/1960 | Back et al.      | 162—83   |
| 2,970,882 | 2/1961  | Kumin et al.     | 8—156 X  |

FOREIGN PATENTS

461,242 11/1949 Canada.

S. LEON BASHORE, Primary Examiner

U.S. CL. X.R.

35 8—111; 162—84